

# UNITED STATES PATENT OFFICE.

LEWIS W. CHUBB, OF EDGEWOOD PARK, PENNSYLVANIA, ASSIGNOR TO WESTINGHOUSE ELECTRIC AND MANUFACTURING COMPANY, A CORPORATION OF PENNSYLVANIA.

## ALLOY.

1,291,408.

Specification of Letters Patent. Patented Jan. 14, 1919.

No Drawing.

Application filed January 2, 1915. Serial No. 177.

*To all whom it may concern:*

Be it known that I, LEWIS W. CHUBB, a citizen of the United States, and a resident of Edgewood Park, in the county of Allegheny and State of Pennsylvania, have invented a new and useful Improvement in Alloys, of which the following is a specification.

My invention relates to metallic alloys, and it has for its object to produce alloys having high magnetic permeability when subjected to the action of strong magnetic fields.

Alloys containing various proportions of nickel and iron, such as the well known nickel-steel, have been prepared in order to produce material which has superior physical properties or which is rust-proof, steam-proof or adapted for use as resistance material. It has also been found that the addition of nickel to steel in certain proportions may render the steel wholly non-magnetic, while, in other proportions, it increases the permeability of the steel at low induction.

I have discovered that the addition of certain percentages of nickel to iron and steel produces alloys having greatly increased permeability, when subjected to strong magnetic fields, in comparison with ordinary iron and steel. This increase in permeability is sufficiently great to render the alloys especially well suited to the manufacture of electric apparatus requiring high magnetic induction, such as rotary converters, direct-current generators and the like.

I have found that the maximum degree of magnetic permeability at high induction may be imparted to iron and steel by the addition of amounts of nickel ranging from 1% to 7% of the alloy. If pure iron, such as that produced electrolytically, is alloyed with nickel, the nickel should constitute about 7% of the alloy, while the amount of nickel added should be changed in accordance with the amounts of other substances, such as carbon, phosphorus, silicon, man-

ganese and sulfur that are present in the iron or steel. For example, when relatively pure iron containing so little additional material as to be substantially pure in a commercial sense, such as the so-called "ingot" iron produced according to U. S. Patents 940,784 and 987,549, is alloyed with nickel, I have obtained the best results when between 2% and 3% of nickel are present. One excellent alloy contained 2.6% of nickel and 97.4% of "ingot" iron. The alloys may be prepared in any convenient and well known manner, and should be annealed before being used.

My improved nickel-steel alloys have good physical properties and a specific gravity somewhat greater than the normal specific gravity of iron. The cost of my alloys is but slightly greater than that of the standard steels now used for magnetic apparatus, and their permeability is very much greater, at high magnetic induction, than that of the standard magnetic steels. Tests upon one sample of nickel-steel prepared according to my invention showed that the nickel-steel had a permeability of 1750, at a magnetic induction of 16,000 gauss, while the best commercial magnetic steels have a permeability below 700 at the same induction. Also, this sample showed a permeability of 335 at 18,000 gauss, while the best commercial steels show only 185 at the same induction.

I claim as my invention:

1. A magnetizable member for use with inductions of 16,000 gauss, or greater, comprising an alloy of from 93 to 99% iron and 7 to 1% nickel.

2. A magnetizable member for use with inductions of 16,000 gauss, or greater, comprising an alloy of from 97 to 98% iron and 3 to 2% nickel.

In testimony whereof, I have hereunto subscribed my name this 24th day of Dec., 1914.

LEWIS W. CHUBB.

Witnesses:

B. B. HINES,  
M. C. MERZ.